# EUROPEAN PATENT SPECIFICATION

(11) **EP 0 185 482 B1**
(45) Date of publication and mention of the grant of the patent: **11.04.1990**
(21) Application number: 85308725.2
(22) Date of filing: 29.11.1985
(51) Int. Cl.: B41M 5/38

(54) **Image receiving element for thermal printers**
Bildaufzeichnungselement für Wärmedrucker
Elément d'enregistrement d'images pour imprimantes thermiques

(30) Priority: 10.12.1984 US 679819
(43) Date of publication of application: 25.06.1986
(73) Proprietor: MINNESOTA MINING AND MANUFACTURING COMPANY, St. Paul, Minnesota 55133-3427 (US)
(72) Inventor: Geisler, Thomas C. c/o Minnesota Mining and, P.O. Box 33427 St. Paul Minnesota 55133 (US); Black, Terrence A. c/o Minnesota Mining and, P.O. Box 33427 St. Paul Minnesota 55133 (US)
(74) Representative: Baillie, Iain Cameron

(56) References cited:
- US-A- 3 941 596
- US-A- 4 032 690
- US-A- 4 181 771
- US-A- 4 218 504

## Description

### Background of the invention

This invention relates to image-receiving elements and their use in the formation of images.

Processes wherein images can be formed by causing a heat-sensitive material to become tacky or fluid in image areas upon imagewise application of heat and then developed by adhering an imaging powder to the tacky image areas are known. An example of such a process is described in U.S. Patent 3,941,596.

Thermal print heads can be used to tackify or fluidize the heat-sensitive material to form the latent image. A simple thermal print head comprises at least one resistance element between two conductors. The thermal print head may also comprise an array of resistance elements. Thus, for example, there may be a 5 by 7 element array on the print head. Additionally, the print head may be fixed or moveable with respect to the surface to be imaged.

The latent image pattern is formed by contacting the resistance element to the heat-sensitive material, providing electric current to the element for a time sufficient to heat the element and raise its temperature to a level sufficient to melt the material in the area of contact, discontinuing the electric current to the element, and relocating the element with respect to the material. The steps of contacting, heating and relocating are repeated until a sufficient number of melted dot-like areas have been provided to define the desired latent liquid image. When the print head has only a single element, the steps necessary to form the latent image must be repeated frequently before an image has been defined. When the print head comprises an array (or matrix) of elements, the steps necessary to form the latent image formation need be repeated fewer times.

A serious problem frequently encountered with thermal print heads is fouling thereof with the heat-sensitive material of the image receiving surface. Generally, the print head is placed in direct contact with the heat-sensitive material. If even a small amount of material from the heat-sensitive coating transfers to the print head and forms a deposit thereon, resolution or image density, or both, is drastically reduced. In many cases, the thermal print heads are not readily accessible for easy cleaning. Some manufacturers of thermal printers recommend passing coarse bond paper through the printer to abrade the deposits from the print head. It is desirable to increase the interval between recommended cleanings of thermal print heads in order to save time and improve resolution.

The image-receiving element of US 3,941,596 comprises a substrate bearing on at least one major surface thereof a coating comprising a) material capable of existing in a supercooled state after melting and subsequent cooling and b) an anti-fouling agent optionally comprising a silica or metal silicate.

### Summary of the invention

The present invention provides an image-receiving element as disclosed in US 3,941,596 characterised in that said anti-fouling agent is selected from the group consisting of wax and a mixture of at least one wax and at least one silica or metal silicate.

Upon being imagewise heated with a thermal print head, a substrate bearing the aforementioned heat-sensitive coating becomes tacky in the image areas. Particles of imaging powder can be adhered to these tackified areas. Optionally, the resulting images can be simultaneously or subsequently fixed.

The advantage of the heat-sensitive coating described is that the thermal print head will avoid being fouled with residue from the coating material, thus assuring formation of images having high resolution for extended periods of use, without the necessity for frequent cleaning of the print head.

Preferred embodiments are defined in the dependent claims.

### Detailed description

The material capable of existing in a supercooled state after melting and subsequent cooling, hereinafter referred to as supercooling material, must have a melting temperature about 10°C above ambient temperature. Ambient temperature, as used herein, refers to the temperature of the environment wherein the imaging process is conducted (e.g., at room temperature of about 19°C to 20°C). The material of the coating must also form a supercooled melt when cooled to a temperature below its melting temperature, i.e. these materials exist, at least temporarily, as fluid metastable liquids after being melted and then cooled below their melting temperatures. When the latent image has been formed, it should wet the surface of the substrate. Moreover, the image must remain fluid and in place until it is contacted with (i.e., developed by) the dry imaging powder. Alternatively, it may be allowed to cool below its melting point to form a supercooled melt before the image areas are developed. Because the supercooled liquid has not regained its solid state, the material retains sufficient memory in the imaged areas to be developed and fixed. Once the material regains its solid state in the imaged areas, the latent image ceases to exist as a distinct area.

Preferably, the supercooling material melts within the approximate range of 40°C to 140°C. Due to the lack in the available chemical literature of adequate data for defining the supercooling materials useful in the practice of the invention, definitive test procedures have been established, one which will now be described.

The melting point or melting range of the supercooling material is determined, for the purposes of this invention, by placing a small amount of the material in powder form on a glass microscope slide, covering the sample with a cover glass, heating the material on a microscope having a hot stage which is provided with temperature measuring means, and observing the temperature at which the particles melt and fuse.

A test for determining if a material is a supercooling material suitable for this invention is conveniently accomplished using the same sample as for the melting point test. A Leitz hot stage microscope having an electrically heated stage which may be cooled by circulation of cold water is used for both determinations. After the stage has been heated above the melting point of the sample, it is cooled and the temperature noted at which crystallization or solidification occurs. Both heating and cooling may be accomplished at somewhat higher rates of temperature change than are ordinarily specified where more precise measurements are required. Materials which when thus treated remain liquid to a temperature well below their melting points, e.g., at least about 60°C below their melting points, have been found to be effective as supercooling materials for this invention; materials which crystallize or solidify at or near their melting points should not be used for making powder-retaining latent images in accordance with this invention. Some materials solidify to a glassy rather than a visibly crystalline state, a condition which is easily determined by applying moderate pressure on the cover glass with a spatula; glassy droplets retain their shape, whereas the liquid droplets flow or rapidly crystallize. A more elaborate test for determination of supercooling materials suitable for this invention is described in U.S. Patent 3,360,367, incorporated herein by reference.

A number of supercooling materials are useful in the coatings of the invention. Representative examples of these materials include dicyclohexyl phthalate, diphenyl phthalate, triphenyl phosphate, dimethyl fumurate, benzotriazole, 2,4 - dihydroxy benzophenone, tribenzylamine, benzil, vanillin, and phthalophenone. Another useful material of this type is "Santicizer 9", a mixture of ortho- and para-toluene sulfonamides commercially available from the Monsanto Chemical Company. Mixtures of these materials are also useful. The supercooling material can also consist of two or more materials that are not supercooling by themselves, but are combinable to form a supercooling material.

The anti-fouling agent can be selected from the following classes of materials:
A. Waxes.
B. Mixtures of waxes with silicas or metal silicates or both.

As used herein, the term "anti-fouling agent" means a material, i.e., a chemical compound or mixture of chemical compounds, that is added to the heat-sensitive composition that inhibits or prevents foreign substances from being deposited on the thermal print head. The materials that are useful as anti-fouling agents in the composition of this invention have at times been referred to as lubricants and antiblocking agents.

Waxes that are suitable for the composition of the present invention include aliphatic alcohols having at least 10 carbon atoms, fatty acids having at least 12 carbon atoms, fatty amides having at least 12 carbon atoms, fatty acid esters having at least 12 carbon atoms, symmetrical ketones derived from fatty acids having at least 12 carbon atoms, metal salts of fatty acids having at least 12 carbon atoms, and fluorocarbon polymers.

Aliphatic alcohols that are suitable for the compositions of this invention can be represented by the formula wherein
R¹ represents a saturated or unsaturated hydrocarbon radical, e.g. alkyl, alkenyl, having 9 to 21 carbon atoms.
Representative examples of such suitable aliphatic alcohols include cetyl, stearyl, lauryl, myristyl, and mixtures thereof.

Fatty acids that are suitable for the compositions of this invention can be represented by the formula wherein
R² represents a saturated or unsaturated hydrocarbon radical, e.g. alkyl, alkenyl, having 11 to 21 carbon atoms.
Representative examples of such fatty acids include palmitic, stearic, lauric, myristic, and mixtures thereof.

Fatty amides that are suitable for the compositions of this invention can be represented by the formula wherein
R² is as defined above, and
X represents or H.

Representative examples of such fatty amides include stearamide, lauramide, oleamide, ethylene - bis - stearamide and mixtures thereof.

Fatty acid esters that are suitable for the compositions of this invention can be represented by the formula wherein
R² is as defined above, and
R³ represents a saturated or unsaturated hydrocarbon radical, e.g., alkyl, alkenyl, having 1 to 22 carbon atoms, said hydrocarbon radical being unsubstituted or substituted with hydroxy group.

Representative examples of such suitable fatty acid esters include glyceryl stearates, e.g. glyceryl monostearate and diethylene glycol monostearate, glycol stearates, cetyl palmitate, stearyl stearate, n-butyl stearate, n-octyl stearate.

Symmetrical ketones that are suitable for the composition of this invention can be represented by the formula wherein
R² is as defined above.

Representative examples of symmetrical ketones derived from fatty acids that are useful in compositions of this invention inlcude stearone and laurone.

Metal salts of fatty acids that are suitable for the compositions of this invention can be represented by the formula wherein
M represents a metal atom,
n represents an integer from 1 to 3, inclusive, and
R² is as defined above.

Metal salts of fatty acids that are suitable for the composition of the present invention include octoates, laurates, palmitates, and stearates of aluminum, lead, cadmium, barium, calcium, lithium, magnesium, and zinc. The metal stearates are most preferred. Blends of metal salts of fatty acids, e.g. zinc stearate, and fatty acids, e.g. stearic acid, are also useful as anti-fouling agents in the composition of the present invention.

One or more of the hydrogen atoms of the hydrocarbon radicals R¹, R², R³ can be replaced with other atoms, e.g., halide, or groups of atoms, e.g. hydroxyl, so long as said atoms or groups of atoms do not adversely affect the anti-fouling characteristics of the wax anti-fouling agent.

Fluorocarbon polymers that are suitable for the composition of the present invention include polymeric tetrafluoroethylene.

Silicas and metal silicates can be used as components of the anti-fouling agent in the composition of the present invention. Representative examples of these materials include silica gel, fumed silica, precipitated silica, clay, kaolin, and talc.

The silicas and metal silicates can be blended with waxes such as for example metal salts of fatty acids, e.g. metal stearates, fluorocarbon polymers, e.g., polytetrafluoroethylene, and fatty amides, e.g. stearamide, which improves their anti-fouling action.

Binders are desirably included in the heat-sensitive composition of the image receiving element. The heat-sensitive composition would tend to flake off under certain conditions in the absence of binders. Representative examples of organic polymeric binders suitable for this invention include water soluble binders such as polyvinyl alcohol, polyvinyl pyrrolidone, hydroxyethyl cellulose, and organic solvent soluble binders such as cellulose acetate, ethyl cellulose, and polyvinyl chloride.

Substrates suitable for use in the invention can be selected from any dry, solid material that is compatible with the coating of normally solid, non-tacky material. Examples of materials suitable for the substrate include polymeric films, metal foils, and paper. The preferred substrate is paper.

The range of concentration of each ingredient in the heat-sensitive coating material has been found to be important. If too little anti-fouling agent is employed, the thermal print heads will become fouled relatively rapidly. If too much anti-fouling agent is employed, the optical density of the toned image will be too low. The ranges of concentration of each ingredient is also dependent upon the nature of anti-fouling agent employed. When waxes are used as the anti-fouling agent, the concentration ranges for essential ingredients of the heat-sensitive coating material are as follows:

When silicas or metal silicates are used in combination with waxes as the anti-fouling agent, the concentration ranges for essential ingredients of the heat-sensitive material are as follows:

The coating material can be applied to the surface of a substrate by a variety of techniques, including both solvent coating and dry coating. For example, the heat-sensitive coating material can be dissolved or dispersed in an appropriate solvent (e.g., acetone, or water), the solution or dispersion applied to the substrate, and the solvent allowed to evaporate. The previously dissolved or dispersed solid material is then allowed to crystallize. Evaporation of the solvent can be accelerated, if desired, by heating the coated substrate. However, care should be taken to insure that the substrate does not curl or otherwise suffer adverse effects as a result of the heating. Additionally, crystallization of the dissolved or dispersed solid material can be accelerated by seeding the coated substrate with like solid material.

Dry coating techniques can also be utilized. The solid form of the heat-sensitive coating material can be brushed or rubbed onto the substrate. Preferably, the solid form of the material is either in the form of a powder or in a form in which it can readily be converted to a powder. The dry coating technique is an efficient means for applying the material to the substrate. Materials applied by the dry coating technique do not soak into the substrate as they do with solvent coating techniques. This is beneficial since it reduces the amount of coating material applied to the substrate while continuing to provide as good an image as that when the coating material is applied by a solvent coating technique. Furthermore, when a plain paper substrate is coated by the dry coating technique, the resultant sheet appears indistinguishable from an uncoated paper sheet and can be used immediately after coating.

The exact amount of the coating material on the substrate can vary. There should be sufficient coating material to form a latent image but not so much material that the thermal printing means is adversely affected, the article becomes too dielectric, or gives a greasy feel or appearance. A sufficient amount of coating material must be used so that once the latent image has been formed, there will be sufficient adhesion between it and the imaging powder to overcome the triboelectric or magnetic forces, or both, holding the imaging powder to the development roll.

It has been found that from about 0.1 to 5 g/m² provides excellent results. When solvent coating is utilized, the substrate preferably bears from 0.1 to 2 g/m² of the material, more preferably from about 0.1 to 1.2 g/m², and most preferably from about 0.2 to 1.0 g/m² of the material. These relatively small amounts of coating material are sufficient to provide latent images that can be developed and essentially permanently fixed to the substrate.

When dry coating techniques are employed, the particulate material is substantially absorbed onto the substrate surface. When the substrate is paper, the material becomes attached to the surface of the paper fibers.

The imaged area must provide sufficient adhesion to the dry imaging powder. The imaged area may react with the imaging powder; it may form a solution with the powder; it may wet the powder; or it may either absorb or be adsorbed by the powder. Whatever the interaction between the powder and the imaged area is, the imaged area must hold the powder until the powder is fixed to the substrate.

Coatings were evaluated by printing a solid bar (0.66 m (26 inches) long) with the thermal print head in the EMT 9140 Facsimile Machine (3M Company). The latent image was then developed with the toner station of a VQC compact copier (3M Company) and toner powder described in U.S. Patent No. 3,925,219, Example 1. The toner particles ranged in size from 10 to 45 micrometers.

The printer utilized a 3.94 styli/mm (100 styli/inch) thick film print head manufactured by Rolm Corporation.

Print head residue was evaluated by visually inspecting the head under 5x magnification and rated according to the following criteria:
None-No visible residue.
Trace-Small specks of coating adhering to print head.
Light-Small amount of residue forming continuous coating on portion of print head, but not interfering with head contact to paper.
Medium-Residue forms continuous coating over approximately half of the print head.
Heavy-Large amount of residue on and behind print head and interfering with head contact to paper and heat transfer.

Image density after development was measured with a MacBeth TR 924 densitometer in reflection mode.

### Examples 1-8

Coating material formulations are set forth in Table I. In the following table the amounts are in parts by weight.

The phthalates and cellulosic binders were dissolved in acetone. The wax anti-fouling agents were dispersed into the phthalate/binder/acetone solution using an ultrasonic bath. The filler anti-fouling agents were dispersed into the phthalate/binder/acetone solution using a homogenizer. The dispersions were coated on paper with a 13 mm (1/2 inch) diameter #8 wire wound rod and air dried, yielding a dry coat weight of 3.01 to 3.88 g/mm² (0.28 to 0.36 g/ft²).

Each coated sheet was evaluated and the results are shown in Table II.

When no anti-fouling agent was present in the heat-sensitive material, print head residue ranged from light to heavy. When at least one anti-fouling agent was included in the heat-sensitive material, print head residue ranged from none to trace.

### Example 9

This example demonstrates the effect of coating weight on printhead residue.

The following formulation was used to prepare test samples:

Samples of the formulation were coated on paper at coating weights ranging from 0.26 g/m² to 0.95 g/m². Coating weight was varied by using different Mayer rods. The results of the printhead residue evaluation are shown in Table III.

From Table III, it can be seen that a dry coating weight of 0.62 g/m² provided optimum optical density value with no print head residue.

### Examples 10-16

These examples demonstrate the effect of different waxes in combination with metal silicate (aluminum silicate) in the coating composition.

The following formulations were used for the examples. In the following table, the amounts are in parts by weight.

Each coating was evaluated and the results are shown in Table V.

## Claims

1. An image-receiving element comprising a substrate bearing on at least one major surface thereof a coating comprising a) material capable of existing in a supercooled state after melting and subsequent cooling and b) an anti-fouling agent optionally comprising a silica or metal silicate characterised in that said anti-fouling agent is selected from the group consisting of wax and a mixture of at least one wax and at least one silica or metal silicate:

2. An image-receiving element according to claim 1 further comprising a binder.

3. An image-receiving element according to claim 1 or claim 2 wherein said anti-fouling agent consists of a wax.

4. An image-receiving element according to any preceding claim wherein said wax is selected from the group consisting of aliphatic alcohols, fatty acids, fatty amides, fatty acid esters, and symmetrical ketones derived from fatty acids.

5. An image-receiving element according to claim 4 wherein said wax is represented by the formula wherein
R¹ represents a saturated or unsaturated hydrocarbon radical having 9 to 21 carbon atoms.

6. An image-receiving element according to claim 4 wherein said wax is represented by the formula wherein
R² represents a saturated or unsaturated hydrocarbon radical having 11 to 21 carbon atoms.

7. An image-receiving element according to claim 4 wherein said wax is represented by the formula wherein
R² represents a saturated or unsaturated hydrocarbon radical having 11 to 21 carbon atoms, and
X represents or H.

8. An image-receiving element according to claim 4 wherein said wax is represented by the formula wherein
R² represents a saturated or unsaturated hydrocarbon radical having 11 to 21 carbon atoms,
R³ represents a hydrocarbon radical having 1 to 21 carbon atoms.

9. An image-receiving element according to claim 4 wherein said anti-fouling agent is represented by the formula wherein
R² represents a saturated or unsaturated hydrocarbon radical having 11 to 21 carbon atoms.

10. An image-receiving element according to any of claims 1 to 3 wherein said wax is a metal salt of a fatty acid.

11. An image-receiving element according to claim 10 wherein said wax is represented by the formula wherein
R² represents a saturated or unsaturated hydrocarbon radical having 11 to 21 carbon atoms,
n represents an integer from 1 to 3, inclusive,
M represents a metal atom.

12. An image-receiving element according to any of claims 1 to 3 wherein said wax is a fluorochemical wax.

13. An image-receiving element according to any of claims 3 to 12 as dependent on claim 2 wherein said material capable of existing in a supercooled state after melting and subsequent cooling comprises 55 weight percent to 99 weight percent of the coating, said wax comprises 1 weight percent to 16 weight percent of the coating, and said binder comprises up to 40 weight percent of the coating.

14. An image-receiving element according to any of claims 4 to 13 as dependent on claim 1 or claim 2 wherein said anti-fouling agent comprises a mixture of a wax and either a silica or a metal silicate.

15. An image-receiving element according to claim 14 wherein said material capable of existing in a supercooled state after melting and subsequent cooling comprises 50 weight percent to 95 weight percent of the coating, said anti-fouling agent comprises 5 weight percent to 40 weight percent of the coating, and said binder comprises 3 weight percent to 40 weight percent of the coating.

16. An image-receiving element according to any preceding claim wherein said material capable of existing in a supercooled state is capable of being supercooled to a temperature at least 60°C below its melting point.

17. An image-receiving element as claimed in any preceding claim wherein said substrate is paper, a polymeric film or a metal foil.

18. A method of preparing an image comprising the steps:
1) providing an image-receiving element according to any preceding claim,
2) heating selected regions of said image-receiving element with a thermal print head to bring said selected regions of said coating to a state in which they can adhere to imaging powder,
3) applying imaging powder to said selected regions to form a developed image on said image receiving element.

## Patentansprüche

1. Bildaufnahmeelement mit einem Substrat, das auf mindestens einer Breitseite einen Überzug trägt, der a) einen Werkstoff enthält, der imstande ist, nach seinem Schmelzen und darauffolgenden Kühlen in einem unterkühlten Zustand zu existieren, und b) ein Antifoulingmittel, das gegebenenfalls mindestens teilweise aus einem Siliciumoxid oder einem Metallsilikat besteht, dadurch gekennzeichnet, daß das Antifoulingmittel aus der Gruppe ausgewählt ist, die aus Wachs und einem Gemisch aus mindestens einem Wachs und mindestens einem Siliciumoxid oder Metallsilikat besteht.

. 2. Bildaufnahmeelement nach Anspruch 1, das ferner ein Bindemittel enthält.

3. Bildaufnahmeelement nach Anspruch 1 oder 2, dadurch gekennzeichnet, daß das Antifoulingmittel aus einem Wachs besteht.

4. Bildaufnahmeelement nach einem der vorhergehenden Ansprüche, dadurch gekennzeichnet, daß des Wachs aus der Gruppe ausgewählt ist, die aus den aliphatischen Alkoholen, den Fettsäuren, den Fettsäureamiden, den Fettsäureestern und den von Fettsäuren abgeleiteten symmetrischen Ketonen besteht.

5. Bildaufnahmeelement nach Anspruch 1, dadurch gekennzeichnet, daß das Wachs durch die Formel dargestellt wird, in der R¹ ein gesättigtes oder ungesättigtes Kohlenwasserstoffradikal mit 9 bis 21 Kohlenstoffatomen darstellt.

6. Bildaufnahmeelement nach Anspruch 4, dadurch gekennzeichnet, daß das Wachs durch die Formel dargestellt wird, in der R² ein gesättigtes oder ungesättigtes Kohlenwasserstoffradikal mit 11 bis 21 Kohlenstoffatomen darstellt.

7. Bildaufnahmeelement nach Anspruch 4, dadurch gekennzeichnet, daß das Wachs durch die Formel dargestellt wird, in der R² ein gesättigtes oder ungesättigtes Kohlenwasserstoffradikal mit 11 bis 21 Kohlenstoffatomen und oder H darstellt.

8. Bildaufnahmeelement nach Anspruch 4, dadurch gekennzeichnet, daß das Wachs durch die Formel dargestellt wird, in der R² ein gesättigtes oder ungesättigtes Kohlenwasserstoffradikal mit 11 bis 21 Kohlenstoffatomen und R³ ein Kohlenwasserstoffradikal mit 1 bis 21 Kohlenstoffatomen darstellt.

9. Bildaufnahmeelement nach Anspruch 4, dadurch gekennzeichnet, daß das Antifoulingmittel durch die Formel dargestellt wird, in der R² ein gesättigtes oder ungesättigtes Kohlenwasserstoffradikal mit 11 bis 21 Kohlenstoffatomen darstellt.

10. Bildaufnahmeelement nach einem der Ansprüche 1 bis 3, dadurch gekennzeichnet, daß das Wachs ein Metallsalz einer Fettsäure ist.

11. Bildaufnahmeelement nach Anspruch 10, dadurch gekennzeichnet, daß das Wachs durch die Formel dargestellt wird, in der
R² ein gesättigtes oder ungesättigtes Kohlenwasserstoffradikal mit 11 bis 21 Kohlenstoffatomen,
n eine ganze Zahl von (einschließlich) 1 bis 3 und
M ein Metallatom darstellt.

12. Bildaufnahmeelement nach einem der Ansprüche 1 bis 3, dadurch gekennzeichnet, daß das Wachs ein fluorchemisches Wachs ist.

13. Bildaufnahmeelement nach einem der Ansprüche 3 bis 12, soweit sie auf den Anspruch 2 rückbezogen sind, dadurch gekennzeichnet, daß.der Überzug zu 99 Gew.-% aus dem Werkstoff besteht, der geeignet ist, nach seinem Schmelzen und darauffolgenden Kühlen in einem unterkühlten Zustand zu existieren, ferner zu 1 bis 16 Gew.-% aus dem Wachs und zu bis zu 40 Gew.-% aus dem Bindemittel.

14. Bildaufnahmeelement nach einem der Ansprüche 4 bis 13, soweit sie auf den Anspruch 1 oder 2 rückbezogen sind, dadurch gekennzeichnet, daß das Antifoulingmittel ein Wachs und entweder ein Siliciumoxid oder ein Metallsilikat im Gemisch enthält.

15. Bildaufnahmeelement nach Anspruch 14, dadurch gekennzeichnet, daß der Überzug zu 50 bis 95 Gew.-% aus dem Werkstoff besteht, der geeignet ist, nach seinem Schmelzen und darauffolgenden Kühlen in einem unterkühlten Zustand zu existieren, ferner zu 5 bis 40 Gew.-% aus dem Antifoulingmittel und zu 3 bis 40 Gew.-% aus dem Bindemittel.

16. Bildaufnahmeelement nach einem der vorhergehenden Ansprüche, dadurch gekennzeichnet, daß der Werkstoff, der geeignet ist, in einem unterkühlten Zustand zu existieren, auf eine Temperatur von mindestens 60°C unter seinem Schmelzpunkt unterkühlbar ist.

17. Bildaufnahmeelement nach einem der vorhergehenden Ansprüche, dadurch gekennzeichnet, daß das Substrat Papier, einen polymere Folie oder eine Metallfolie ist.

18. Verfahren zum Herstellen eines Bildes mit folgenden Schritten:
a) es wird ein Bildaufnahmeelement nach einem der vorhergehenden Ansprüche verwendet,
b) ausgewählte Bereiche des Bildaufnahmeelements werden mit einem Thermodruckkopf derart erwärmt, daß die ausgewählten Bereiche des Überzuges in einen Zustand gelangen, in dem sie an einem Bildpulver haften können,
c) durch Aufbringen von Bildpulver auf die ausgewählten Bereiche wird auf dem Bildaufnahmeelement ein entwickeltes Bild erzeugt.

## Revendications

1. Elément d'enregistrement d'images comprenant un substrat portant au moins sur une de ses surfaces principales un revêtement comprenant a) une matière capable d'exister à l'état surfondu après fusion puis refroidissement et b) un agent anti-encrassement comprenant facultativement une silice ou un silicate métallique, caractérisé en ce que ledit agent anti-encrassement est choisi parmi l'ensemble constitué par une cire et un mélange d'au moins une cire et d'au moins une silice ou un silicate métallique.

2. Elément d'enregistrement d'images selon la revendication 1 comprenant de plus un liant.

3. Elément d'enregistrement d'images selon la revendication 1 ou la revendication 2, dans lequel ledit agent anti-encrassement est constitué d'une cire.

4. Elément d'enregistrement d'images selon l'une quelconque des revendications précédentes, dans lequel ladite cire est choisie parmi l'ensemble constitué par les alcools aliphatiques, les acides gras, les amides gras, les esters d'acide gras et les cétones symétriques dérivées d'acides gras.

5. Elément d'enregistrement d'images selon la revendication 4, dans lequel ladite cire est représentée par la formule dans laquelle R¹ représente un radical hydrocarboné saturé ou insaturé ayant de 9 à 21 atomes de carbone.

6. Elément d'enregistrement d'images selon la revendication 4, dans lequel ladite cire est représentée par la formule dans laquelle R² représente un radical hydrocarboné saturé ou insaturé ayant de 11 à 21 atomes de carbone.

7. Elément d'enregistrement d'images selon la revendication 4, dans lequel ladite cire est représentée par la formule dans laquelle R² représente un radical hydrocarboné saturé ou insaturé ayant de 11 à 21 atomes de carbone, et
X représente ou H.

8. Elément d'enregistrement d'images selon la revendication 4, dans lequel ladite cire est représentée par la formule dans laquelle
R² représente un radical hydrocarboné saturé ou insaturé ayant de 11 à 21 atomes de carbone, et
R³ représente un radical hydrocarboné ayant de 1 à 21 atomes de carbone.

9. Elément d'enregistrement d'images selon la revendication 4, dans lequel ledit agent anti-encrassement est représenté par la formule dans laquelle R² représente un radical hydrocarboné saturé ou insaturé ayant de 11 à 21 atomes de carbone.

10. Elément d'enregistrement d'images selon l'une quelconque des revendications 1 à 3, dans lequel ladite cire est un sel métallique d'un acide gras.

11. Elément d'enregistrement d'images selon la revendication 10, dans lequel ladite cire est représentée par la formule dans laquelle
R² représente un radical hydrocarboné saturé ou insaturé ayant de 11 à 21 atomes de carbone,
n est un entier valant de 1 à 3 inclusivement, et
M représente un atome métallique.

12. Elément d'enregistrement d'images selon l'une quelconque des revendications 1 à 3, dans lequel ladite cire est une cire fluorochimique.

13. Elément d'enregistrement d'images selon l'une quelconque des revendications 3 à 12, dans la mesure où elles sont dépendantes de la revendication 2, dans lequel ladite matière capable d'exister à l'état surfondu après fusion, puis refroidissement, constitue 55% à 99% du poids du revêtement, ladite cire constitue 1 % à 16% du poids du revêtement et ledit liant constitue jusqu'à 40% du poids du revêtement.

14. Elément d'enregistrement d'images selon l'une quelconque des revendications 4 à 13, dans la mesure où elles dépendent de la revendication 1 ou de la revendication 2, dans lequel ledit agent anti-encrassement est constitué d'un mélange d'une cire et soit d'une silice, soit d'un silicate métallique.

15. Elément d'enregistrement d'images selon la revendication 14, dans lequel ladite matière capable d'exister à l'état surfondu après fusion, puis refroidissement, constitue 50% à 95% du poids du revêtement, ledit agent anti-encrassement constitue 5% à 40% du poids du revêtement et ledit liant constitue 3% à 40% du poids du revêtement.

16. Elément d'enregistrement d'images selon l'une quelconque des revendications précédentes, dans lequel ladite matière capable d'exister à l'état surfondu peut être surfondue à une température inférieure d'au moins 60°C à son point de fusion.

17. Elément d'enregistrement d'images selon l'une quelconque des revendications précédentes, dans lequel ledit substrat est un papier, une pellicule polymère ou une pellicule métallique.

18. Procédé pour préparer une image comprenant les stades consistant à:

1) faire appel à un élément d'enregistrement d'images selon l'une quelconque des revendications précédentes,

2) chauffer des régions choisies dudit élément d'enregistrement d'images avec une tête d'impression thermique pour porter lesdites régions choisies dudit revêtement dans un état où elles peuvent adhérer à une poudre formatrice d'images,

3) appliquer une poudre formatrice d'images auxdites régions choisies pour former une image développée sur ledit élément d'enregistrement d'images.
